

## 1

3,520,785

### ELECTROPLATING GOLD AND THIOMALATE ELECTROLYTE THEREFOR

Robert Duva, 646 Terrace Drive, Paramus, N.J. 07652, and John P. Raleigh, 218 Pulaski St., Dunellen, N.J. 08812

No Drawing. Continuation-in-part of application Ser. No. 584,679, Oct. 6, 1966. This application Apr. 14, 1969, Ser. No. 816,067

Int. Cl. C23b 5/42, 5/28

U.S. Cl. 204—43

4 Claims 10

#### ABSTRACT OF THE DISCLOSURE

Bright gold electrodeposits are obtained from an aqueous alkaline bath containing gold, added as alkali metal gold thiomalate, and a minute proportion of a soluble arsenic compound.

This application is a continuation-in-part of U.S. application Ser. No. 584,679 filed Oct. 6, 1966, of the same title, now abandoned.

This invention relates to a process and electrolyte for plating of bright gold.

Among the objects of the invention is to provide an electrolyte and process for plating bright gold.

Among other objects of the invention is to provide a process and electrolyte for plating bright 24 karat gold.

The objects of the invention are attained by dissolving a gold thiomalate complex in an alkaline solution to provide an electrolyte containing a dissolved alkali metal gold thiomalate complex, adding a minute amount of arsenic to said bath (as a soluble salt) and adjusting the pH to about 10 to 12.

The bath is operated at a temperature of about 24°—82° C. and at a current density of 2—10 amperes/ft.<sup>2</sup>.

The arsenic is added in proportions of approximately 10 mg. to 0.12 gm. per liter of solution and can be added in the form of any arsenic compound which is soluble in the bath at the said pH range of 10 to 12. Since the bath is alkaline, the alkali metal arsenites and the various alkali metal arsenates are well suited as the addition compounds. The arsenic can also be added to the bath in the form of the oxide or the halide in which case an alkali metal arsenite or arsenate is formed with the alkali of the bath.

Processes of electroplating metals including gold by passing an electric current through a bath containing mercapto-metal complex salts are disclosed in U.S. 3,238,112 and among the mercapto compounds which form said metal complexes, 2-mercaptopsuccinic acid (thiomalic acid) is disclosed. Without the arsenic addition as disclosed in the present application, gold deposited from the alkali metal gold thiomalate complex is, at most, semi-bright when thicknesses of 100  $\mu$ " are approached. ( $\mu$ "-microinches)

Alkali metal gold thiomalates can be made by the process described in U.S. 1,994,213 or by the process of U.S. 3,238,112.

The preferred ranges of components and conditions for obtaining bright gold deposits are as follows:

Thiomalic acid—40—100 g./l. (preferably 45—52 g./l.)

Alkali hydroxide—25—60 g./l.

Gold (as alkali metal gold thiomalate)—4—8 g./l.

As (as soluble compound)—10 mg. to 0.12 g./l. (preferably 10—30 mg./l.)

## 2

pH—10—12

Temperature—24—82° C.

Current density—2—10 amps/ft.<sup>2</sup>

Bright gold deposits can be obtained with more than 5 30 mg./l. of arsenic, but the additional arsenic does not increase the brightness.

The following example is given to illustrate, in detail, a preferred embodiment of the invention, but it will be understood that the invention may be otherwise embodied within the scope of the broader claims.

#### EXAMPLE

An aqueous solution of thiomalic acid in sufficient proportions to provide 52 g. of the acid is mixed with an aqueous solution of sodium hydroxide in sufficient proportions to provide 40 g. of NaOH. Approximately 8 g. of previously formed sodium gold thiomalate is dissolved in the resultant mix and water is added to make 1 liter. Approximately 35 mg. of sodium arsenite (or sufficient 15 to provide about 20 mg. of As) is added to the solution. The pH of the bath is measured and adjusted to pH 11.5, if necessary, by the addition of NaOH or thiomalic acid. Products plated from the bath at a temperature of 70° C. and current density of 2 amps/ft.<sup>2</sup> (voltage 0.7) are 20 bright in thicknesses as high as 500 $\mu$ " or more.

We claim:

1. An aqueous alkaline electroplating bath for the deposition of bright gold consisting essentially of the following ingredients in the proportions set forth:

Thiomalic acid—40—100 g./l.

Alkali hydroxide—25—60 g./l.

Gold (as alkali metal gold thiomalate)—4—8 g./l.

Arsenic (as a soluble compound)—10 mg. to 0.12 g./l.

2. The bath of claim 1 wherein the arsenic is added in 25 the proportion of 10—30 mg./l.

3. A process for the electroplating of bright gold comprising electrolyzing an aqueous solution containing the following ingredients in the proportions set forth:

Thiomalic acid—45—52 g./l.

Alkali hydroxide—25—40 g./l.

Gold (as sodium gold thiomalate)—6—8 g./l.

Arsenic (as a soluble compound)—10 mg. to 0.12 g./l.

pH—10—12

45 at a current density of 2—10 amps/ft.<sup>2</sup> and a temperature of 24—82° C.

4. The process as claimed in claim 3 wherein the arsenic is present in the proportion of 10—30 mg./l.

#### References Cited

##### UNITED STATES PATENTS

3,238,112 3/1966 Haslam ----- 204—46 XR  
3,423,295 1/1969 Greenspan ----- 204—43

##### FOREIGN PATENTS

55 1,027,637 2/1953 France.

##### OTHER REFERENCES

60 Edmund R. Thews, Metal Finishing, pp. 80—85, September 1951.

Francis C. Frary, Transactions of the Electrochemical Society, vol. 23, pp. 25—97 (1913).

JOHN H. MACK, Primary Examiner

65 G. L. KAPLAN, Assistant Examiner

U.S. Cl. X.R.

204—46